

Aug. 8, 1933.

R. N. HARTZELL

1,921,184

METHOD OF MAKING VENEER AND A NEW ARTICLE OF VENEER

Filed Feb. 25, 1931

2 Sheets-Sheet 1

FIG. 1.



INVENTOR  
Robert N. Hartzell.  
BY *Toulman & Toulman*  
ATTORNEYS.

Aug. 8, 1933.

R. N. HARTZELL

1,921,184

METHOD OF MAKING VENEER AND A NEW ARTICLE OF VENEER

Filed Feb. 25, 1931

2 Sheets-Sheet 2



*Robert N. Hartzell*  
INVENTOR  
BY  
*Bauman & Bauman*  
ATTORNEYS.

## UNITED STATES PATENT OFFICE

1,921,184

METHOD OF MAKING VENEER AND A NEW  
ARTICLE OF VENEERRobert N. Hartzell, Piqua, Ohio, assignor to  
Hartzell Industries, Inc., Piqua, Ohio, a Cor-  
poration of Ohio

Application February 25, 1931. Serial No. 518,169

10 Claims. (Cl. 144—309)

My invention relates to a process of making veneer, particularly veneer of multiple kinds of woods; it further relates to a process of producing a veneer, preferably of multiple woods, 5 in circular or substantially square sheets.

It is my object to provide a very cheap and permanent veneer out of relatively cheap materials and small size materials built up into composite work pieces from which the veneer is 10 cut producing the effect of inlaid work that can only be otherwise secured by the most expensive hand labor and from the most expensive woods.

It is a further object to provide a new article 15 of manufacture for use as veneer in which the multiple pieces of different kinds of wood are so interlocked one with the other as to make it possible to retain the several parts in engagement despite the expansion and contraction of 20 the several pieces of wood.

Referring to the drawings:

Figure 1 is a plan view of a complete sheet of veneer formed of multiple woods interlocked with one another;

25 Figure 2 is a section on the line 2—2 of Figure 1;

Figure 3 is a section on the line 3—3 of Figure 1;

30 Figure 4 is a side elevation of the tapered work piece as it has been cut down during the process of cutting the veneer from the end of the work piece with the result shown in Figure 1;

Figure 5 is an end elevation showing the edges 35 of the inserts of different wood from the main body of veneer work piece;

Figure 6 is a view of the side opposite to 40 Figure 4 showing the location of one of the inserts;

Figure 7 is a top plan view of the multiple work piece.

The veneer in question is cut from the work piece in accordance with the machine and process of my application Serial No. 511,238, filed 45 January 26, 1931, although I do not desire to confine my present invention to any particular machine, as different types of veneer can be cut from the present work piece of my invention with different machines according to the nature 50 of the veneer produced.

In producing my work piece, I take air-dried lumber designated at 1, 2 and 3, which has about 55 15 to 25 percent moisture in it. I coat the adjacent faces of these pieces 1, 2 and 3 with glue, such as casein glue 4, and place between

the glued surfaces another wood which is dry, being substantially moisture free, such wood being designated 5. The part 5 is relatively drier than the parts 1, 2 and 3 so it can absorb the moisture from the glue and then have about 60 the same relative amount of moisture that the other parts have. I prefer a wood that is relatively soft compared to the pieces 1, 2 and 3, but that is not absolutely essential.

This dry veneer insert 5 absorbs the moisture 65 in the glue, bringing about a permanent setting of the parts in engagement with one another. I then soak the entire work piece in hot water bringing the temperature thereof up to 150 to 200 degrees Fahrenheit.

70 I then cut the work piece into the veneer strips or pieces, such as is shown in Figure 1, while hot.

As the tapered end of the work piece is cut away into veneer, it leaves the waste end 6. 75 The hole 7 merely indicates a place for receiving one of the holding fingers to maintain the work piece in position, and forms no part of the present invention.

It will be noted that, in the cutting of this 80 sheet of veneer with the interleaved pieces of different kinds of wood, a regular design is thus provided, as will be seen in Figure 1.

It will also be noted from Figure 3 that the 85 plane of juncture between the strips 5 and the pieces 1, 2 and 3, as at 8, is at an angle to the top 9 and the bottom 10 of the veneer sheet shown in Figure 1.

Due to this overlapping, there can be an expansion and contraction between the two types 90 of wood without complete separation, thereby making it possible to have a very thin sheet in which the several parts are retained in engagement with one another without cracking, splitting and loss of the inserts which is not possible where the juncture surfaces 8 are vertical to the surfaces 9 and 10.

It will be understood that I desire to comprehend within my invention such modifications as 100 may be necessary to adapt it to varying conditions and uses.

Having thus fully described my invention, what I claim as new and desire to secure by Letters Patent, is:

1. In a method of making a work piece for veneer, air drying portions of the work piece, coating the surfaces thereof with an adhesive, inserting between the adhesive surfaces a relatively drier strip of wood.

2. In a method of making a work piece for

veneer, air drying portions of the work piece, coating the surfaces thereof with an adhesive, inserting between the adhesive surfaces a relatively drier strip of wood, and subjecting the composite strip to a temperature of water of approximately 150 to 200 degrees Fahrenheit.

3. In a process of making a work piece for veneer, coating an air dried strip of lumber with adhesive, applying a moisture free strip of lumber thereto, and absorbing the moisture from the adhesive by the moisture free strip.

4. In a process of making veneer, coating an air dried strip of lumber with adhesive, applying a relatively drier strip of lumber thereto, absorbing the moisture from the adhesive by the last-named drier strip, and soaking the composite strip in hot water until it attains a temperature of approximately 150 to 200 degrees Fahrenheit, and cutting the veneer strip therefrom while the work piece so formed is still subject to the temperature applied to it.

5. In a process of making a work piece for veneer, air drying a piece of wood until the moisture content of 15 to 25 percent remains, applying to the surface thereof an adhesive, applying to the adhesive a relatively drier piece of wood, absorbing the moisture in the adhesive by the last-named drier piece of wood.

6. In a process of cutting veneer, air drying a piece of wood until the moisture content of 15 to 25 percent remains, applying to the surface thereof an adhesive, applying to the adhesive a relatively drier piece of wood, absorbing the moisture in the adhesive by the last-named drier piece of wood, and soaking the work piece thus formed in water until it attains a temperature of approximately 150 to 200 degrees Fahrenheit.

40

80

85

90

95

100

105

110

ROBERT N. HARTZELL.

115

45

120

50

125

55

130

60

135

65

140

70

145

75

150

7. In a process of cutting veneer, air drying a piece of wood until the moisture content of 15 to 25 percent remains, applying to the surface thereof an adhesive, applying to the adhesive a relatively drier piece of wood, absorbing the moisture in the adhesive by the last-named drier piece of wood, soaking the work piece thus formed in water until it attains a temperature of approximately 150 to 200 degrees Fahrenheit, and cutting veneer strips therefrom while hot.

8. In a process of making veneer, air drying a piece of wood until it has 15 to 25 percent moisture content, applying adhesive to one surface thereof, and applying a relatively soft relatively drier piece of wood to said adhesive.

9. In a process of making a work piece for veneer, air drying a piece of wood until it has 15 to 25 percent moisture content, applying adhesive to one surface thereof, applying a relatively soft relatively drier piece of wood to said adhesive, said soft strip being relatively thinner than the first mentioned piece of air dried wood.

10. In a process of making veneer, forming a work piece by air drying one portion thereof until it has 15 to 25 percent moisture content, applying casein glue to the surface thereof, applying a relatively drier soft wood to the surface of said glue, absorbing the moisture from the glue by the last-named drier piece of wood, soaking the composite work piece thus formed in hot water until it attains a temperature of from 150 to 200 degrees Fahrenheit, and cutting while hot into veneer strips.